

Jan. 8, 1957

W. E. MARSHALL ET AL

2,776,883

PROCESS AND APPARATUS FOR SMELTING IRON WITH MOBILE FUELS

Filed Aug. 7, 1953



INVENTOR.  
WILLIAM E. MARSHALL  
AND SAMUEL A. BELL,  
BY

*Allen & Allen*  
ATTORNEYS.

1

2,776,883

## PROCESS AND APPARATUS FOR SMELTING IRON WITH MOBILE FUELS

William E. Marshall and Samuel A. Bell, Middletown, Ohio, assignors to Armco Steel Corporation, Middletown, Ohio, a corporation of Ohio

Application August 7, 1953, Serial No. 373,008

18 Claims. (Cl. 75—48)

This invention relates to an apparatus for smelting iron with mobile fuels. In the copending application of Marshall, Serial No. 226,231, filed May 14, 1951, there is disclosed a process and apparatus for reducing and smelting iron. According to that teaching, a flame is produced in a bath-type furnace from a mobile fuel, the flame having a temperature of at least 3,000° F. and the products of combustion of the flame being reducing to iron oxide. The heat from the flame maintains the bath of iron in molten condition in the furnace and the products of combustion of the flame, which are of reducing character, are used outside the furnace proper to reduce finely divided iron ore and the iron and the gangue and then melted inside the furnace by the heat of the flame. A flame which has a sufficiently high temperature and, nevertheless, yields products of combustion reducing to iron may be provided by the use of oxygen or oxygen enriched air for purposes of combustion and by preheating of the mobile fuel or the oxygen or oxygen enriched air or both.

The term "mobile fuel" in said application and in the present application is used to mean natural and artificial combustible gases such as, natural gas, methane, ethane, propane, butane, ethylene, acetylene, hydrogen and the like which contain as their principal combustion components hydrogen or hydrocarbons (but without more than a minor concentration of gases containing combined oxygen such as carbon monoxide and water vapor), and also to mean oil or other liquid hydrocarbon fuels and solid pulverized carbonaceous fuels such as powdered coal, coke, or carbon black. The process there disclosed makes it possible to operate with substantial economy particularly where a plentiful supply of cheap mobile fuel is available. Since the iron ore is used in finely divided condition, a cheaper ore may be used and it is unnecessary to use coke either as a fuel or as a skelton in a shaft furnace.

In another copending application of Marshall, Serial No. 264,859, filed January 4, 1952, certain improvements were disclosed. According to the last mentioned application, the iron was smelted by means of mobile fuels by a method in which the iron ore was reduced directly in the furnace in which the molten bath of iron and slag was being maintained by the flame. This procedure is designated as fluo-solid reduction. Improvements were taught in connection with a more economical utilization of the heat generated in the process.

In both these copending applications, the addition of coke to the molten bath is used where it is wished to lower the melting point of the iron and where it is desirable to lower the percent of iron oxide in the slag to a very low value. It is an object of the present invention to provide a process and apparatus suitable for carrying out the melting step of the combined reduction and melting process, in which the carbon content of the iron can be increased effectively and in a manner economical of coke.

2

It is another object of the present invention to provide an apparatus which is simple and relatively inexpensive to construct, by means of which a very small amount of coke is consumed in the production of iron in relation to the coke requirements of a conventional blast furnace.

These and other objects of the invention which we shall describe in greater detail hereinafter or which will become apparent to one skilled in the art to which it pertains, upon reading these specifications, we accomplish by that certain construction and arrangement of parts of which we shall now disclose certain exemplary embodiments.

Reference is made to the drawings forming a part hereof and in which:

Figure 1 is a somewhat diagrammatical cross sectional view through one form of apparatus according to the invention.

Figure 2 is a fragmentary view similar to Figure 1 showing a modification.

Figure 3 is a plan view of a modified apparatus.

Figure 4 is a cross sectional view taken on the line 4—4 of Figure 3, and

Figure 5 is a cross sectional view of still another modification.

In attempting to increase the carbon content of the molten metal bath produced by the new process of the copending applications previously described, by the addition of coke, coal, gas carbon, or other carbonaceous substances, certain complications arise. The products of combustion of the flame in the melting furnace, while reducing to iron, are highly oxidizing to all forms of carbon and will result in its partial combustion and consequent waste.

Furthermore, these products of combination, which include water vapor, are highly decarburizing to iron and will tend to remove carbon from the molten bath nearly as fast as it is being added. This makes it difficult to attain desired values of carbon in the molten iron without the excessive and uneconomical use of coke or other solid carburizing substances.

Briefly, in the practice of our invention we provide a combustion chamber having a burner, preferably at the top thereof, and we supply the burner with mobile fuel, as described above, together with oxygen or oxygen enriched air in proper proportions, and carrying entrained in said mobile fuel reduced iron ore in finely divided form and slag forming constituents such as gangue and CaO. The iron and slag making constituents melt in the combustion chamber and flow down the floor or overflow preferably through a portion of a coke filled tower into a bath-type furnace or collecting hearth having an enclosed coke column thereabove. While we have specifically referred to coke herein, it must be understood that our teachings apply with equal force to equivalent materials, including non-coking coals, anthracite coal, char produced from coal during synthesis gas production, and other solid carbonaceous materials. A stack is provided to lead away the products of combustion from the combustion chamber without their passing through the coke column. Means may be provided to bring oxygen or oxygen enriched air to the coke column to burn a minor amount of the coke in order to control hearth temperature, if necessary, and to aid in starting up the unit.

Referring more particularly to Figure 1, a combustion chamber is indicated at 10 and is shown as having the sloping floor 11. A burner is diagrammatically indicated at 12 to which are fed the mobile fuel, oxygen or oxygen enriched air, finely divided entrained reduced iron ore, gangue, and CaO. The fuel burns in the combustion chamber 10 and the products of combustion pass in the direction of the arrows through the stack 13, while

the slag forming constituents and the iron melt and collect on the floor 11. A relatively shallow aperture 14 is provided for the passage of the molten materials and the products of combustion. A bath-type furnace or collecting hearth is indicated at 15 and is provided with a coke containing chamber 16. The sloping floor 11 communicates with the collecting hearth by means of a shallow aperture 17 through which the molten materials flow into the collecting hearth 15 through a portion of the coke in the coke chamber 16. The bath of molten iron is indicated at 18, the slag layer at 19, and the coke at 20. A tap hole for the iron is provided at 21 and, if desired, a tap hole may be provided at 22 for the slag. These holes are closed in the well known manner with clay plugs 23 and 24. A duct 25 is shown through which oxygen or oxygen enriched air is fed to the coke column to burn some of the coke to control the temperature in the hearth and to maintain the bath in molten condition.

In connection with the materials fed to the burner 12, it will be understood that the finely divided iron ore has been previously reduced by any suitable reduction process. The natural gas or other mobile fuel and the oxygen or oxygen enriched air are supplied in such proportion that the atmosphere of combustion products in the chamber 19 will be non-oxidizing to iron, i. e. reducing to  $FeO$ , and the temperature generated in the combustion will be such that the iron, gangue, and  $CaO$  will melt and collect on the sloping bottom of the chamber.

It will be observed that the bridge wall 13a between the combustion chamber and the stack brings about a complete reversal of direction of gas travel. This tends to throw out the solids which are entrained in the gases from the combustion chamber 10. The iron and slag in liquid form run down the inclined bottom 11 through the apertures 14 and 17 and are collected in the collecting hearth 15 in separate layers of molten iron 18 and molten slag 19. The bottom 11 may be level or even hollowed to form a pool which overflows through the aperture 17.

It will also be observed that the coke 20 in the column 16 is preheated through the wall 13b between the coke column and the stack. Furthermore, since the iron and slag enter the coke column at a temperature which is well above their melting points, and since the melting point of the iron is further substantially lowered by dissolving carbon, it will be clear that very little, if any, air or oxygen is used at the tuyere 25 and very little coke is consumed in order to maintain the slag and the iron liquid in the hearth. As a matter of fact with a large furnace where the heat loss per unit of product is very small, the tuyere 25 is seldom used except for starting the process.

Coke consumption can be reduced still further, as shown in Figure 2, by causing the oxygen or oxygen enriched air supplied to the tuyere 25 to pass through a preheater, generally indicated at 26.

Whereas a conventional blast furnace consumes about 1800 pounds of coke per ton of iron produced, an apparatus according the present disclosure producing several hundred tons of iron a day consumes very little coke. Substantially just enough coke is consumed to saturate the iron with carbon. On very small experimental furnaces operating at low production rates, the coke consumed amounts to about 400 pounds to a ton of iron, but on a very large furnace, as outlined above, the coke consumption will approach a low of about 100 pounds per ton.

In certain parts of the country where natural gas is very cheap and coke is relatively expensive, great savings can be effected in the manufacture of pig iron by the use of the apparatus herein disclosed. As a matter of fact, pig iron may be manufactured entirely independently of metallurgical coke or natural gas if powdered bituminous coal is substituted for natural gas in the

burner 12 and if hard anthracite coal, gas carbon, etc., is used in the place of coke in the column 16.

In addition to providing a passage for the flow of molten iron and slag into the hearth of the furnace at 15, the aperture 17 also decreases the area of contact between the coke and the gases in the combustion chamber and stack. These gases contain a considerable amount of water vapor as well as a little  $CO_2$  which would oxidize some of the coke and greatly increase its consumption if the combustion chamber gases were permitted to have unlimited contact with the coke. The top of the coke chamber being closed by openable bells, slide valves, or the like, the relatively small amounts of  $CO$  and  $N_2$  from the combustion taking place at tuyere 25 pass out through the slot 17 and join the body of gas passing through the stack 13, so that if the slot 17 is kept shallow the velocity of the gases passing toward the left of the aperture 17 prevent contact of water vapor and  $CO_2$  with the coke. The aperture 17 therefore constitutes a very important feature of the invention in that it prevents the decarburizing gases from coming into contact with the coke. The products of combustion at tuyere 25 are not decarburizing and will consume only the amount of coke needed to provide any extra heat needed to hold the molten metal at the desired temperature, or to bring the furnace up to operating temperature when starting up.

In Figure 2, we have also illustrated how the slot 17a may be positioned in a slightly different manner from that shown in Figure 1. The slot 17a, however, performs the same functions as the slot 17.

In Figures 3 and 4, we have shown an arrangement amounting, in effect, to a battery of devices according to Figure 1 having a common hearth and coke column 35 fed by two or more combustion chambers and provided with two or more stacks. In Figure 4, we have shown the combustion chambers 10a and 10b having the burners 12a and 12b and the stacks 13c and 13d. The coke column is indicated at 16a and the hearth at 15a. The tuyeres 25a and tap hole 21a may be as in Figure 1.

In Figure 5, we have shown a slightly different arrangement in which the gases pass out to a stack at the opposite side of the combustion chamber from the coke column. Here the combustion chamber is indicated at 10c. The fuel, entrained solids and oxygen are fed through the pipe 12c. An additional pipe 12d has been provided, through which additional solids may be fed, as desired. The metal melted in the chamber 10c flows over the sloping floor 11a as before through an aperture or slot 17b into the hearth 15b. The coke column 16b again contains a body of coke 20 and again a tuyere 25b is provided. The molten iron layer is shown at 18 and the slag layer at 19 and the molten metal may be cast through the tap hole 21b.

In this instance, however, the stack 13e is on the opposite side of the combustion chamber and the products of combustion pass out through a slot 14a in a direction opposite to that in which the molten metal flows. We have merely shown the embodiment of Figure 5 as a feasible modification, but we prefer the embodiments of Figures 1 to 4, inclusive, because the coke column is more effectively preheated by its proximity to the products of combustion.

In the claims which follow, we have used the word "oxygen" in a sense inclusive of impure oxygen (which commercially may contain as much as 5% nitrogen) and of oxygen enriched air.

It will be understood that many modifications may be made without departing from the spirit of our invention and that we do not intend to limit ourselves except as set forth in the claims which follow.

Having now fully described our invention, what we claim as new and desire to secure by Letters Patent is:

1. An apparatus for the purpose described comprising a combustion chamber, a burner opening into said cham-

ber, means for conducting mobile fuel, oxygen, entrained reduced iron ore, and slag-forming constituents in finely divided form, through said burner, a bath-type furnace having an enclosed coke chamber extending thereabove, and a stack opening from said combustion chamber for carrying away the products of combustion, and an aperture opening from the lower part of said combustion chamber through which molten iron and slag may flow into said furnace.

2. The structure of claim 1 in which tuyere means are provided for supplying oxygen to the coke chamber at a point above the hearth of the bath-type furnace.

3. The structure of claim 2 in which means are provided for preheating the oxygen supplied to said coke chamber.

4. The structure of claim 1 in which the aperture from the combustion chamber enters the coke chamber at a distance above the hearth of the bath-type furnace, whereby the molten iron passes through a portion of the coke in the coke chamber.

5. An apparatus for the purpose described, comprising a combustion chamber, a burner at the top of said chamber, means for supplying a mobile fuel, oxygen, entrained reduced iron ore and slag-forming constituents in finely divided form to said burner, said chamber having a sloping floor extending to a bath-type furnace having an enclosed coke chamber thereabove, a shallow aperture between said sloping floor at its lowest point and a wall of said combustion chamber through which molten iron and slag may flow over said sloping floor into said bath-type furnace, means for supplying oxygen to said coke chamber, and a stack adjacent said combustion chamber for carrying away the products of combustion.

6. The structure of claim 5 in which means are provided for preheating the oxygen supplied to said coke chamber.

7. An apparatus for the purpose described, comprising a combustion chamber, a burner at the top of said chamber, means for supplying a mobile fuel, oxygen, and entrained reduced iron ore and slag-forming constituents in finely divided form to said burner, said chamber having a sloping floor and a shallow aperture between said chamber floor at its lowest point and a wall of said chamber, a stack for carrying away the products of combustion, and a bath-type furnace having an enclosed coke chamber thereabove, said sloping floor continuing under said stack to said furnace, a shallow aperture between said stack and furnace with which said sloping floor communicates at its lowest point, the heat of the products of combustion being transmitted to the coke in said coke chamber to preheat the same, and means for supplying oxygen to said coke chamber.

8. The structure of claim 7 in which means are provided to preheat the oxygen supplied to said coke chamber.

9. An apparatus for the purpose described, comprising a combustion chamber, a stack, and a bath-type furnace having an enclosed coke chamber thereabove in juxtaposition in the order named, a sloping floor for said combustion chamber extending on a downward slope under said stack and to said furnace, a shallow aperture between said floor and the wall separating said combustion chamber and stack, a second shallow aperture between said floor and the wall separating said stack and furnace, through which molten metal and slag may flow from said combustion chamber under said stack and into said furnace, the products of combustion passing from said combustion chamber to said stack through the first named aperture, means for supplying oxygen to said coke, a burner at the top of said combustion chamber, and means for supplying to said burner a mobile fuel, oxygen, and entrained finely divided reduced iron ore and slag-forming constituents.

10. The structure of claim 9 in which means are provided for preheating the oxygen supplied to said coke chamber.

11. The structure of claim 9 wherein said furnace constitutes the central element of the apparatus and a plurality of said combustion chambers and stacks are radially disposed with respect thereto, whereby said plurality of chambers feed a common furnace.

12. A structure according to claim 11 wherein means are provided to preheat the oxygen supplied to said coke chamber.

13. An apparatus for the purpose described, comprising a combustion chamber, a burner at the top of said combustion chamber, means for supplying to said chamber a mobile fuel, oxygen, and entrained finely divided reduced iron ore and slag-forming constituents, said chamber having a sloping floor, a bath-type furnace having an enclosed coke chamber thereabove adjacent said combustion chamber, a shallow aperture between said floor and the wall separating said combustion chamber and furnace whereby molten iron and slag may flow over said floor from said combustion chamber into said furnace, a stack adjacent said combustion chamber, a shallow aperture between said floor and the wall separating said combustion chamber and stack through which the products of combustion may pass, and means for supplying oxygen to said coke chamber.

14. The structure of claim 13 wherein means are provided for preheating the oxygen supplied to said coke chamber.

15. A process of smelting iron while minimizing iron losses in the slag, which comprises entraining finely divided iron in a mobile fuel, burning said fuel in a combustion chamber with an oxygen bearing gas richer in oxygen than air, under conditions productive of a temperature of about 3000° F. and of products of combustion which are reducing to iron, causing the molten iron to pass out of said combustion chamber and into a collecting hearth through a body of carbonaceous material in solid form to lower the melting point of the iron and to enrich the iron in carbon, and removing the products of combustion while preventing their contact with said carbonaceous solid material.

16. A process according to claim 15 wherein the finely divided iron is provided by causing the products of combustion of said mobile fuel to produce a fluo-solid reduction of finely divided iron oxide ore.

17. A process according to claim 15 including the step of maintaining the temperature of the molten iron in said collecting hearth by controlled combustion of a portion of said carbonaceous material in solid form with an oxygen bearing gas richer in oxygen than air.

18. A process of smelting iron in finely divided condition, which comprises producing in a combustion chamber with a mobile fuel a flame having a temperature of about 3000° F., the products of combustion of which within the said combustion chamber and at substantially the melting point of iron will be sufficiently reducing to iron oxide to prevent reoxidation of finely divided reduced iron introduced into said combustion chamber with said mobile fuel, and to effect reduction of incompletely reduced iron oxide if present, causing the molten iron to pass out of said combustion chamber and into a collecting hearth through a body of carbonaceous material in solid form to lower the melting point of the iron and to enrich the iron in carbon, and removing the products of combustion while preventing their contact with said carbonaceous solid material.

#### References Cited in the file of this patent

#### UNITED STATES PATENTS

|           |            |               |
|-----------|------------|---------------|
| 538,004   | Williamson | Apr. 23, 1895 |
| 1,512,262 | Allingham  | Oct. 21, 1924 |
| 1,524,182 | Kjolberg   | Jan. 27, 1925 |

#### FOREIGN PATENTS

|         |               |               |
|---------|---------------|---------------|
| 157,295 | Great Britain | Apr. 10, 1927 |
|---------|---------------|---------------|